

# UNITED STATES PATENT OFFICE.

WALTER KAEMPF, OF GROSSENHAIN, GERMANY.

## PROCESS FOR THE MANUFACTURE OF OIL-VARNISH SUBSTITUTES FROM ANIMAL-OILS.

1,087,064.

Specification of Letters Patent.

Patented Feb. 10, 1914.

No Drawing.

Application filed July 19, 1912. Serial No. 710,423.

To all whom it may concern:

Be it known that I, WALTER KAEMPF, a subject of the Emperor of Germany, and residing at Grossenhain, in Saxony, Germany, have invented certain new and useful Improvements in Processes for the Manufacture of Oil-Varnish Substitutes from Animal-Oils, of which the following is a specification.

10 This invention relates to the treatment of animal oils, such as fish oil train oil or the like, for the purpose of obtaining therefrom suitable constituents for the manufacture of a linseed oil varnish substitute, using 15 superheated steam.

The invention consists in a process in which the animal oil is first treated in a distillation retort or vessel for about two hours at a temperature of 235-240°, and then 20 ejected directly to a distillation by means of steam at about 375-400°, which is blown through the oil mass for about 25-30 hours. The temperature of the contents of the retort is preferably not raised above 260°. 25 After the process is finished the retorts must be emptied at once, access to the air being avoided, as otherwise a gelatinizing of the product may occur. The entire process thus 30 consists of a physical combined with a chemical operation.

In the first stage the uncombined saturated acids are removed from the animal oils by means of the superheated steam, and in the second stage at a certain temperature 35 and after a certain period the superheated steam causes a fractional decomposition, in which the glycerids of the saturated fatty acids separate out and distil over, while the glycerids of the unsaturated acids polymerize and remain in this form. The properties 40 of the linseed oil varnish substitute obtained in this manner are as follows. The product has the odor of heavy oil and is transparent, clear, and elastic even in the 45 cold. Its drying power is considerably higher than that of linseed oil. Deposits of any kind (fatty acids) do not occur even on cooling to 15°. The product can also be used in the making of oil lacquers (copal lacquer) or used as a drying agent or linoxyn 50 substitute. The distillation products consist mainly of fatty acids and glycerin, which can be directly used in the soap and candle making industries.

Several examples of the improved process 55 will now be given.

First example: 10 hundredweights of train oil with the highest possible iodin number, are heated in the distillation vessel for two hours at a temperature of 60 235-240°. The distillation is then at once commenced by passing steam at 375-400° through the oil mass, the temperature of the contents of the retort not being allowed however to rise above 260°. Particular care 65 should be exerted in this respect. After 25 hours the operation is finished. With train oils of low iodin number the process may last 30 hours. In the first hours and up to the 20th the fatty acid distils clear and 70 liquid, and after the 20th hour to the end of the operation the distillation becomes gradually slower, and occurs in white flakes.

Second example: The process of the present invention can be better carried out, and 75 yields a higher output, when conducted partly under a vacuum, or at least a partial vacuum. The more rapid operation obtained with this procedure can be attributed to the fact that the glycerids distil partly 80 undecomposed under a vacuum.

The vacuum may be readily maintained at the same time the steam is blown through the retort for distillation purposes, provided the suction effect of the vacuum pump 85 or other means for providing the vacuum is sufficient to overcome the steam inlet admission, that is to say, provided the suction carries away a larger quantity of air or steam than that which is allowed to enter 90 the retort from the boiler in a given time. By controlling the steam inlet, the vacuum can be regulated as desired.

In carrying out the process the temperature in the retort is maintained at 270 to 95 285°. The maintaining of this temperature is of essential importance as if it falls below this figure the distillation is appreciably retarded and if the said temperatures are exceeded, there is a danger of approaching too closely to the decomposition temperature at which a breaking up of the varnish forming glycerids begins, so that the output is substantially diminished.

The following procedure is also of prime 100 importance in the carrying out of the invention: On removing the finished product from the retort no air should be allowed to

enter owing to the danger of gelatinizing. This danger is very real, because the correct instant for the interruption of the distillation is difficult to recognize and the period of distillation fluctuates greatly owing to the different origins of the animal oils treated. According to the present invention these difficulties are obviated in the most simple manner, by adding fatty acids or their esters to the contents of the retort while the proportion of saturated fatty acids present therein is still small, these added substances acting as distribution or diluting agents and being sluggishly or not at all fluid. The acids of the unsaturated series, for example linoleic acid have proved very suitable, also resin may with advantage be employed.

Another important modification of the improved process consists in treating the train oil, previously heated in any manner, with for example superheated steam of about 375 to 400°, the contents of the retort being kept at 270 to 285°, and carrying on the operation not to completion, but interrupting it as soon as the formation of oil varnish begins. Since in this case saturated acids are still present in the retort contents, these latter must be subjected to a subsequent heating up to 315° so that these fatty acids may still evaporate. The heavy oil becomes continuously more viscid and finally gelatinizes if the heating is too prolonged. To avoid this contingency the necessary amount (5% upward) of fatty acids or their esters can be added during the subsequent heating, in the same way as during the distillation.

Having now described my invention what I claim as new and desire to secure by Letters Patent is:—

1. A process for the manufacture of a linseed oil varnish substitute consisting in preliminarily heating animal oils for a number of hours to a temperature of from 235° to 240° C., subjecting the oils to distillation by means of steam at a temperature of from 375° to 400° C., and maintaining the oil mass during such distillation below the decomposition temperature of the glycerids.

2. A process for the manufacture of a linseed oil varnish substitute consisting in preliminarily heating animal oils for a number of hours to a temperature of from 235° to 240° C., subjecting the oils to distillation under vacuum by means of steam at a temperature of from 375° to 400° C., and maintaining the temperature of the oil mass during such distillation below the decomposition temperature of the glycerids.

3. A process for the manufacture of a linseed oil varnish substitute consisting in preliminarily heating animal oils for a number of hours to a temperature of from 235°

240° C., subjecting the oils to distillation by means of steam at a temperature of from 375° to 400° C. blown through the retort, maintaining the temperature of the oil mass during such distillation below the decomposition temperature of the glycerids, and adding fatty acids to the oil mass when the amount of saturated fatty acids contained therein becomes small.

4. A process for the manufacture of a linseed oil varnish substitute consisting in preliminarily heating animal oils for a number of hours to a temperature of from 235° to 240° C., subjecting the oils to distillation by means of steam at a temperature of from 375° to 400° C. blown through the retort, maintaining the temperature of the oil mass during such distillation below the decomposition temperature of the glycerids, interrupting the distillation when the oil mass contains saturated fatty acids and subsequently heating the contents of the retort to a temperature of about 315° C.

5. A process for the manufacture of a linseed oil varnish substitute consisting in preliminarily heating animal oils for a number of hours to a temperature of from 235° to 240° C., subjecting the oils to distillation under vacuum by means of steam at a temperature of from 375°-400° C. blown through the retort, maintaining the temperature of the oil mass during such distillation below the decomposition temperature of the glycerids, interrupting the distillation when the oil mass contains saturated fatty acids, subsequently heating the contents of the retort to a temperature of about 315° C., and adding fatty acids during such subsequent heating.

6. A process for the manufacture of a linseed oil varnish substitute consisting in preliminarily heating animal oils for several hours to a temperature of from 235° to 240° C., subjecting the oils to distillation under vacuum by means of steam at a temperature of from 375° to 400°, and maintaining the temperature of the oil mass during such distillation at from 270° to 285°.

7. A process for the manufacture of a linseed oil varnish substitute consisting in preliminarily heating animal oils for a number of hours to a temperature of from 235° to 240° C., subjecting the oils to distillation by means of steam at a temperature of from 375° to 400°, maintaining the oil mass during such distillation at from 270° to 285°, and adding fatty acids to the oil mass when the amount of saturated fatty acids contained therein becomes small.

8. A process for the manufacture of a linseed oil varnish substitute consisting in preliminarily heating animal oils for a number of hours to a temperature of from 235° to 240° C., subjecting the oils to distillation

by means of steam at a temperature of from 375° to 400°, maintaining the oil mass during such distillation at from 270° to 285°, interrupting the distillation when the oil 5 mass contains saturated fatty acids and subsequently heating the mass to about 315° C.

In testimony whereof I have signed my name to this specification in the presence of two subscribing witnesses.

WALTER KAEMPF.

Witnesses:

PAUL ARRAS,  
CLARE SIMON.